

(No Model.)

No. 272,900.

J. REESE.

COMPOUND ORDNANCE.

4 Sheets—Sheet 1.

Patented Feb. 27, 1883.



WITNESSES

Walter Reese  
John Smythe

INVENTOR

Jacob Reese  
By  
Franklin Reese, Jr.

(No Model.)

4 Sheets—Sheet 2.

J. REESE.

COMPOUND ORDNANCE.

No. 272,900.

Patented Feb. 27, 1883.



Witnesses

Ja<sup>ck</sup> Rees<sup>e</sup>.

Thos. Longf<sup>th</sup>

Inventor

Jac<sup>ob</sup> Rees<sup>e</sup>.

by  
Frank M. Rees<sup>e</sup>, Atty.

(No Model.)

4 Sheets—Sheet 3.

J. REESE.

COMPOUND ORDNANCE.

No. 272,900.

Patented Feb. 27, 1883.



Witnesses  
Master Reese.  
John Smith  
L.W.

Inventor  
Jacob Reese  
by  
Frank M. Reese, City

(No Model.)

J. REESE.

4 Sheets—Sheet 4.

No. 272,900.

COMPOUND ORDNANCE.

Patented Feb. 27, 1883.



witnesses.

Hezekia Reese.  
Thos. Smith  
W.

Inventor.

Jacob Reese,  
by Frank W. Reese, Atty

# UNITED STATES PATENT OFFICE.

JACOB REESE, OF PITTSBURG, PENNSYLVANIA.

## COMPOUND ORDNANCE.

SPECIFICATION forming part of Letters Patent No. 272,900, dated February 27, 1883.

Application filed January 16, 1882. (No model.)

To all whom it may concern:

Be it known that I, JACOB REESE, residing at Pittsburgh, in the county of Allegheny and State of Pennsylvania, have invented a certain new and useful Improvement in the Manufacture of Cannon; and I do hereby declare the following to be a full, clear, and exact description thereof, reference being had to the accompanying drawings, forming a part thereof, in

10 which—

Figure 1 on Sheet 1 indicates a plan view of a solid cylindrical cast-steel ingot. Fig. 2 on Sheet 1 indicates a plan view of the same after it has been welded and rolled or hammered down to the required size to form a solid homogeneous internal structure for a cannon, and after it has been turned at one end, so as to be readily centered in a mold for casting the cast-steel or cast-iron jacket of the cannon around it. Fig. 3 on Sheet 1 indicates a sectional longitudinal view of the jacket after being cast around the rolled or hammered steel cylinder. Fig. 4 on Sheet 1 indicates a longitudinal section of the gun after it is bored to form a breech-loader, the dotted lines indicating the thickness of the walls of the interior solid, hammered, or rolled tube formed by boring the hammered or rolled steel ingot. Fig. 1 on Sheet 2 indicates a ground plan of a muzzle-loading gun when finished. Fig. 2 on Sheet 2 indicates a longitudinal section of the same. Fig. 3 on Sheet 2 indicates an end view of the same. Fig. 1 on Sheet 3 indicates a vertical section of the gun-mold, with the solid hammered or rolled cast-steel cylinder adjusted in position in the center of the mold. Fig. 1 on Sheet 4 indicates a ground plan of the casting-pit, with the gun-mold and the core-heating furnace in place. Fig. 2 on Sheet 4 indicates a sectional elevation of a gas heating-furnace with the hammered or rolled cast-steel core or cylinder adjusted in position for previous heating before being inserted in the casting-mold. Fig. 3 on Sheet 4 indicates a side view of a portion of the gun core or ingot and of a shield for adjusting the upper portion of the core into the center of the mold, and also to permit a portion of the metal to flow out of the upper part of the mold, so as to secure a sound and solid top to the gun in casting.

Like letters of reference indicate like parts wherever they occur.

My invention relates to the manufacture of ordnance or cannon; and it consists, first, in a new and useful method of producing a cast-steel or cast-iron gun having a perfect weld or union with a dense, solid, and homogeneous hammered or rolled core-barrel; second, in an improved apparatus adapted to the use of my invention, and, third, in the improved product.

The objects are, first, to secure a close, dense, and homogeneous solid structure in that portion of the steel which forms the walls of the bore; secondly, to form a perfect welding or union of the core-barrel with the body of the gun; thirdly, to obviate the necessity for the employment of the costly and cumbersome machinery now in use for the manufacture of steel ordnance; and, fourthly, to improve the quality and reduce the cost of manufacture.

It is a well-known fact to all metallurgists that steel ingots and castings have a cellular or porous structure, and, on the other hand, that cast-iron may be produced comparatively free from this defect. The reasons for this are, carbon, silicon, and phosphorus exert a marked influence on the fusing-point of iron. The higher they are the lower will be the fusing-point of the metal, the greater the fluidity of the metal at any given temperature, and the longer it will remain in a fluid condition after being cast. Cast-iron contains a large percentage of these impurities. Hence it will melt at a comparatively low temperature, may be raised to a high degree of fluidity, and will remain in a fluid state for a considerable length of time after it is cast. Hence there is ample time and the proper conditions for the escape, after casting, of any gases which may be occluded in the metal, and consequently a sound casting may be produced. In the manufacture of steel, however, almost all of these impurities are removed by chemical action, and a large quantity of the gases resulting from this action is occluded in the metal, and as the proportion of the impurities is low the steel requires a high temperature to maintain it in a fluid condition, sets quickly after being cast, and sufficient time or the proper conditions cannot be secured to allow the escape of the occluded gases after the metal has been cast. In order to overcome this defect, it has been usual to cast the ingot and then subject it to a forging operation to bring it to the size and

shape required for the gun. This, however, produces an imperfect result, as large masses frequently contain cavities, and have a cellular internal structure even after having been subjected to the most careful and skillful manipulation. The most effective system of hammering proves inefficient when applied to large masses, in consequence of the fact that the inertia of the mass attacked will often cause the effect of the blow to be felt only near the exterior, the internal structure remaining after treatment nearly as spongy and irregular as before. Another defect of this system of treating large masses of steel is, that it is necessary to subject the metal to repeated sectional heatings, which also tend to prevent a uniform physical structure.

From the preceding matter it will be readily understood that the hammering or compressing operation tends to produce a close, solid, and homogeneous physical structure at and near the exterior of the mass, while it has but little effect upon the physical structure of the interior. Consequently ordnance produced by hammering from a large ingot would be liable to be porous and spongy at the walls of the bore. It is necessary, however, that the bore should be of a close and uniform structure, free from cells and soft or hard spots, in order that the friction on the periphery of the ball or projectile in its passage out of the gun may be uniform, so that in its flight the ball or projectile will travel in a line parallel with the bore of the gun; and in order to secure these requisites I propose to produce the guns or ordnance by a method consisting, essentially, of the following steps: I first cast an ingot of any suitable quality of steel, and hammer it down into a cylinder about from two to six inches greater in diameter and from two to six feet longer than the proposed diameter and length of bore in the finished gun. The hammered core is placed in a suitable mold, and the body of the gun is then formed by casting the molten metal around the central core, and when the gun is cold it is withdrawn from the mold, bored, and finished in the usual manner, so that in this case a perfect weld of the core to the body of the gun is had, and the dense, solid, and homogeneous structure of the exterior part of the hammered ingot is secured at the walls of the bore.

In the practice of this method of treatment I am enabled to solidify and render the metal of the core-ingot perfectly homogeneous to the depth of from three to four inches from the surface by the use of comparatively light compressing or hammering machinery, and by placing the hammered or compressed cylinder in the mold and running the molten metal into it a perfect weld, known to the trade as a "teeming" weld, is produced between the core and the body of the gun, and as the central core is of a larger diameter than the bore the walls of the bore will be composed of hammered or compressed steel, of from one to three

inches in thickness, welded perfectly to the body of the gun.

I shall now describe my invention more fully, so that others skilled in the art to which it appertains may make and use the same.

In the drawings, A indicates a plan view of the casting-pit, (see Sheet 4,) with the cannon-mold and gas-heating ingot-furnace in place within it.

B indicates the core-ingot adjusted in position in the center of the mold.

B' indicates an annular opening at the top of the mold to allow the excess of metal to flow up out of the mold.

b indicates the flare of the hopper at the central portion of the upper part of the mold.

b' indicates the walls of the hopper.

b<sup>2</sup> indicates the outside line of the base of the central hopper.

b<sup>3</sup> indicates the spout of the central hopper, through which the excess of metal may flow off.

c indicates the gates through which the metal is run into the mold.

d indicates the flare of the gate-hoppers, and d' their metallic rims.

E indicates the cap of a gas heating-furnace, which is situated in the casting-pit at one side of the flask or mold. This gas heating-furnace is of a cylindrical form, and is provided with an air and gas inlet flue, e, at its lower portion, and an outlet, e', which opens into a waste-gas flue, e<sup>2</sup>, which runs to a waste-gas stack, e<sup>3</sup>.

e<sup>4</sup> indicates adjusting-screws for adjusting the hammered ingot or core in the center of the gas heating-furnace.

In Fig. 1 on Sheet 3, F indicates face-plates, which are formed of tile of the required size, and placed in the bottom of the gates, to prevent the molten metal from cutting the bottom of the gates when poured into them.

f indicates the openings at the bottom of the gates to allow the metal to run into the mold, and f' indicates the annular openings between the gates and the mold which form the trunions.

G indicates the annular opening between the core and the mold to form the body of the gun.

H indicates the bearing-ribs, which are planed true, so that the sections of the mold may fit true and tightly together; and H' indicates the depressions in the flask adjoining the ribs, in order to prevent the mold from warping.

It will be noticed by reference to Sheet 3 that the annular spaces which form the trunions of the gun communicate with the gates. The idea of this is to allow a portion of the metal to flow from the gates into the mold through the trunion-openings, and thus secure greater soundness at the trunions.

When a gun of, say, ten-inch bore and twelve feet in length is to be produced, I cast an ingot of any suitable quality of steel about twenty inches in diameter and of sufficient

weight to form a core, when hammered, of the length desired. The ingot is then heated and hammered down to about from fourteen to sixteen inches in diameter, and one of its ends is beveled off, as shown in Fig. 3 on Sheet 1, so that it may be afterward readily centered in the casting-mold. The hammered core is then conveyed to the casting-pit, and the cap of the core-heating furnace is removed, and the core is lowered down and arranged in its center. The cap of the furnace is then replaced, and gas and air are admitted into the core-heating furnace until the core is properly heated, when they are shut off, the cap of the furnace is removed, and the mold having been prepared, the core is withdrawn from the furnace and deposited and adjusted in the center of the mold. The steel or cast-iron is then caused to flow into both of the gates in a steady continuous manner until the molten metal arises to and flows out of the central hopper at the top of the flask. The pouring or quantity of metal caused to flow in should be reduced to a less degree at this point, but should be continued to cause the slag and impurities which rise to the top of the metal to flow out of the hopper, in order that a sound upper portion of the casting may be produced. After the outer shell of the casting has solidified, the bolts which unite the mold-sections should be loosened somewhat, to enable the gun to shrink, and the casting-pit should be covered and hermetically sealed and allowed to remain until the gun is cool, when it may be withdrawn, placed in a lathe, and the trunnions turned, and it is then bored and finished in the usual manner.

By this method I am enabled to produce any size, kind, or form of steel guns having a close, dense, and solid texture of the metal at the walls of the bore, having the walls of the bore welded perfectly to the main body of the gun, and possessing a tensile strength of from fifty to one hundred and fifty thousand pounds per square inch of the cross-section, the tensile strength being relative to the percentage of carbon combined with the steel; and I am also able to produce a stronger cast-iron gun than has heretofore been made, as it will possess a close, dense, solid internal structure composed of hammered steel welded perfectly to the cast-iron main body of the gun.

The steel core may be made of crucible, open-hearth, or Bessemer cast-steel, and the main body of the gun may be made of either cast-steel or cast-iron, as desired, as in either case a perfect union with the red-hot steel core may be had; but as cast-iron cannot be relied on to resist a rupturing strain of over thirty thousand pounds to the square inch, and as steel can be readily made to sustain four times this amount of strain, I prefer to construct the gun entirely of steel.

In the practice of the invention I prefer to use steel produced by the "basic process," as it can be made of a purer and tougher quality

than by the use of any other process known to me.

The advantages of the invention are, first, the walls of the bore have a close, dense, and homogeneous texture, free from air-cells or porosity; secondly, as the walls of the bore are of hammered cast-steel, perfectly united or welded to the main body of the gun, they cannot be loosened by contraction and expansion during the use of the gun; third, as the gun is but one single body of steel, or of steel and cast-iron, (when finished,) it will resist greater internal strains, because they will be more uniformly distributed; fourth, as the entire gun may be made of a single mass of the same quality of steel, its expansion and contraction will be more uniform during service, its strength will be more uniform, and its liability to rupture during service greatly decreased; fifth, the walls of the bore will be more uniform in texture than if the whole gun were hammered, as the comparatively small size and the regular form of the core-ingot enable it to be hammered at one heat, whereas the gun would require a series of sectional reheatings, which would produce internal strains; sixth, a better and cheaper gun can be produced, as the walls of the bore will be solid, and the machinery and labor necessary for hammering its irregular shape can be dispensed with; seventh, guns or ordnance can be produced readily and quickly with the machinery now in use in this country for other purposes, thus avoiding the necessity of building a costly plant to work the invention.

I am aware that it has been proposed to cast ordnance in successive layers, forging each layer separately while hot, and do not herein claim the same, for the reason that by such a method the separate layers are subjected to a series of unequal heatings and strains, which destroy the uniform character of the metal or its homogeneity, and the metal immediately surrounding the bore is not compressed, as in the present invention.

Having described my invention, what I claim, and desire to secure by Letters Patent, is—

1. The method herein described of manufacturing cannon, which consists, essentially, in casting a cast-steel ingot or core, hammering the same until its porosity is reduced externally and a homogeneous external shell is formed thereon, casting the metal which forms the body of the gun thereon, and finally boring out the center of the compressed core, substantially as and for the purpose specified.

2. A gun the lining of which is composed of hammered steel and the outer body of a single casting of metal cast upon it, substantially as set forth.

JACOB REESE.

Witnesses:

FRANK M. REESE,  
WALTER REESE.